

## UNITED STATES PATENT OFFICE.

MAX BIELEFELDT, OF KALK, NEAR COLOGNE, GERMANY.

## EXPLOSIVE COMPOUND.

SPECIFICATION forming part of Letters Patent No. 340,276, dated April 20, 1886.

Application filed October 22, 1885. Serial No. 180,583. (No specimens.)

*To all whom it may concern:*

Be it known that I, MAX BIELEFELDT, a citizen of Germany, and resident at Kalk, near Cologne, Germany, have invented new and useful Improvements in Explosive Compounds, of which the following is a specification.

This invention is based on the fact that in the production of explosives by means of nitrated substances the nitro-glycerine can with advantage be wholly or partly replaced by a solution of nitrate of ammonia in water of ammonia. The impregnation of nitro-cellulose with this solution may be effected in the most complete manner by placing the nitro-cellulose, in small quantities at a time, on a hopper-sieve to which a shaking movement is imparted while the solution is continuously poured over it in a fine stream through a rose. The residue that remains on the sieve after this operation should be crushed and treated again in the same manner. The water of ammonia employed should be concentrated to twenty-five per cent., and be of a specific gravity 0.9983 to 0.9709. The process differs according to the rapidity of action or strength of the explosive to be manufactured—that is to say, if a quickly exploding compound or a more slowly exploding but more powerful compound is required.

To produce the most powerful explosive, nitro-glycerine is mixed with nitrated wood-cellulose containing as small as possible an amount of resinous matter. The sawdust of pine wood which has been well freed from resin, or, better still, alder-wood or lime-tree sawdust, which is naturally free from resin, is put, in small quantities at a time, into nitro-glycerine, the sawdust in a perfectly dry condition having been previously moistened with a little ammonia.

Soft nitro-wood-celluloses deprived of resin possess the property, unlike other woody substances, of combining with nitro-glycerine when heated by a water bath, forming a plastic mass which can be easily worked up into cartridges.

The energy of the explosive may be reduced by using a smaller quantity of nitro-glycerine in the manufacture of the explosive.

In order that the material shall possess sufficient coherence and plasticity for making cartridges, I proceed as follows: A weighed quantity of nitro-glycerine is mixed with a corresponding quantity of nitrated wood-cellulose which has previously absorbed a solution (up to fifty per cent.) of equal parts of nitrate of ammonia in water of ammonia of about one to twenty-five per cent. By this means two advantages are obtained: first, a firm and coherent cartridge may be made which contains only thirty per cent. of nitro-glycerine, and yet possesses an energy equal to a Kieselguhr dynamite containing seventy-five per cent. of nitro-glycerine, this result being due to the perfect combustion which ensues on explosion; second, the ammonia has a neutralizing action on the wood-cellulose, which is important when pine wood sawdust which has not been entirely freed from resin and acid is used. The nitro-wood-cellulose prepared as above is now mixed with nitro-glycerine in the usual manner, and the cartridges prepared therefrom. Collodion-cotton may be added; but this is quite unnecessary.

As already mentioned, according to this invention, a reduced quantity of nitro-glycerine may be used or may be entirely dispensed with, and even in the latter case the explosive is much more powerful than compressed blasting powder.

The relative amounts of the constituents of this new explosive differ according to the purpose for which it is destined; but the following may be taken as an average:

(a) When nitro-glycerine is used: nitro-glycerine, .75 to one per cent.; nitrated wood-cellulose, twenty-five to ninety-five per cent.; nitrate of ammonia, one to twenty-five per cent.; water of ammonia, one to twenty-five per cent.; and accessory substances, nitrated cotton-wool, (collodion-cotton,) ten to twenty per cent.

(b) Without nitro-glycerine: nitrated wood-cellulose, forty-five per cent.; nitrated cotton-wool, (collodion-cotton,) five per cent.; nitrate of ammonia, twenty-five per cent.; water of ammonia, twenty-five per cent.

The explosive substance prepared according to this invention, and containing the same or

a less quantity of nitro-glycerine than Kieselguhr dynamite of seventy-five per cent. nitro-glycerine, possesses a much more powerful action than the latter, burns completely, leaving no residue, produces a less quantity of injurious gas, and is less sensitive to dampness, cold, and percussion than the Kieselguhr compositions and other modern explosives.

When this new explosive (which I term "ammonia cellulose dynamite") contains seventy-five per cent. nitro-glycerine, it is almost equal to pure blasting-gelatine.

It being possible to reduce the nitro-glycerine to one per cent., or even to dispense with it altogether, the explosive force may be considerably varied.

Having thus described my invention and the manner of employing the same, I claim—

1. An explosive mixture consisting of nitro-cellulose in a solution of nitrate of ammonia in water of ammonia, as set forth.

2. An explosive mixture consisting of nitro-glycerine and nitro-cellulose with nitrate of ammonia in water of ammonia, as specified.

In testimony whereof I have signed my name to this specification in the presence of two subscribing witnesses.

MAX BIELEFELDT.

Witnesses:

JAS. HENNER,  
ARTHUR OTTO.